

# United States Patent Office

3,597,338

Patented Aug. 3, 1971

1

3,597,338

## METHOD AND ELECTROLYTE FOR ANODIC OXIDATION COATING OF ALUMINUM

Shin Matsuyama and Takekuni Kobayashi, Osaka, Japan, assignors to Minolta Camera Kabushiki Kaisha, Minamiku, Osaka, Japan

No Drawing. Filed July 15, 1969, Ser. No. 842,030

Claims priority, application Japan, Jan. 17, 1969,  
44/3,522

Int. Cl. C23b 9/02

U.S. CL. 204—58

6 Claims

## ABSTRACT OF THE DISCLOSURE

In the anodic oxidation coating of aluminum and its alloys an electrolyte is employed comprising an aqueous solution containing, by weight of said solution, 1% to 30% acetamide, 0.1% to 10% oxalic acid and 0.01% to 0.5% sulphuric acid or its molar equivalent of a water soluble sulphate compound. Deeper colors are achieved at lower voltages and power consumptions.

## BACKGROUND OF THE INVENTION

The present invention relates generally to improvements in metal treating and it relates particularly to an improved method for the production of integrally colored anodic oxidation coatings on articles of aluminum and alloys thereof and an improved electrolyte composition therefor.

The conventional process for forming a colored anodic oxidized coating on articles of aluminum or aluminum alloys includes the step of immersing the aluminum article, which defines an anode, and a cathode defining electrode into an electrolyte, generally sulfuric acid, and applying a voltage between the article and cathode to effect the formation of an oxide coating on the article. However, the resulting coating is greatly deficient because of its high porosity a consequence of which is a low corrosion resistance. Moreover, an additional separate dye treating step is required. The conventional aluminum anodizing procedure accordingly leaves much to be desired. The applicant has found that many of the drawbacks of the conventional aluminum anodizing methods are overcome by employing as an electrolyte an aqueous solution of acetamide and oxalic acid. While this process produces a hard, non-porous, highly corrosion resistant, colored coating on the aluminum article and obviates the need of any additional dye treatment it possesses certain disadvantages, it requires the use of relatively high voltage and is accordingly accompanied by a relatively high power consumption and the resulting color, although variable depending on the composition of the aluminum alloy, is of relatively pale or light hue.

## SUMMARY OF THE INVENTION

It is a principal object of the present invention to provide an improved method and composition for the treatment of metals.

Another object of the present invention is to provide an improved method and composition for the production of anodic oxidation coatings on surfaces of aluminum and alloys thereof.

Still another object of the present invention is to provide an improved method and composition for producing on aluminum containing articles a hard highly corrosion resistant, colored, anodic oxidation coating.

A further object of the present invention is to provide an improved single step method of the above nature characterized by a relatively low voltage requirement and power consumption, great versatility and adaptability, a wide range of colors and depths of color, and a superior resulting coating.

2

In a sense the present invention is based on the discovery that the use, in the formation of an anodic oxidation coating on an aluminum containing surface, of an electrolyte comprising an aqueous solution containing, in addition to acetamide and oxalic acid, a small amount of sulfuric acid or a water soluble sulfate compound which provides sulfate ions in the aqueous solution, produces a hard, nonporous, highly corrosion resistant, deeply colored coating on the aluminum surface, and the voltage requirements between the aluminum surface and the cathode are greatly reduced with a corresponding reduction in power consumption. The present invention accordingly contemplates an electrolyte for the anodic oxidation of aluminum and alloys thereof comprising an aqueous solution of acetamide, oxalic acid, and sulfuric acid or a water soluble sulfate or a combination thereof, as well as the method of treating an aluminum containing work piece comprising immersing the work piece and another electrode in the improved electrolyte and applying a voltage between said work piece and said electrode of a value sufficient to form an oxidation coating on said work piece.

The concentration of the sulfate ion in the aqueous electrolyte solution should be sufficient to reduce the anodic oxidation coating voltage, advantageously to an initial voltage of less than 70 volts and a final voltage of less than 100 volts, and advantageously constitutes by weight of the electrolyte of 0.01% and 0.5% sulfuric acid or its molar equivalent of a water soluble sulphate compound or a combination thereof with sulfuric acid, that is between about 0.01% and 0.5% of the sulfate ion. Preferably the electrolyte contains between 0.1 and 2.0 grams sulfuric acid per liter of electrolyte or the molar equivalent thereof of the sulfate compound or of said compound in combination with sulfuric acid. The electrolyte advantageously contains, by weight, 1% to 50% acetamide, preferably 30 to 200 grams acetamide per liter of electrolyte, and 0.1% to 10% oxalic acid, preferably 3 to 30 grams oxalic acid per liter of electrolyte. The temperature of the electrolyte in the anodizing procedure, the current density and the anodizing time may be greatly varied depending on the desired coating, and the optimum parameters are easily and readily determined by one skilled in the art. Thus an electrolyte temperature between 15° C. and 25° C. and a current density of the order of 2 a./dm.<sup>2</sup> has been found to be highly satisfactory. The color of the anodic oxidation coating is dependent on the composition of the aluminum alloy of the article being treated.

The present invention is characterized by an increased efficiency consequent to a reduction in the required anodizing voltage and in the power consumption and results in a significant reduction in equipment and costs. The improved process is capable of producing a very wide range and depth of colors without the need of separate dyeing steps. The color of the resulting coating is highly resistant to light and weathering and exhibits very little discoloration even when exposed for long periods to out-of-door influences and environments. Thus, articles coated by the present process possess such high wear and corrosion resistance properties that they are highly suitable for outdoor uses and applications.

## DESCRIPTION OF THE PREFERRED EMBODIMENTS

An electrolyte of the following composition was prepared:

|                    | Grams/liter |
|--------------------|-------------|
| Acetamide          | 80          |
| Oxalic acid        | 10          |
| Sulfuric acid      | 0.6         |
| Water <sup>1</sup> | Balance     |

<sup>1</sup> 1 liter in total amount.

The solution prepared in accordance with the above composition was put into an electrolytic cell. Into this solution were immersed a work piece defining aluminum plate to be treated which served as an anode and another aluminum plate which served as a cathode. Three different types of aluminum were employed as the work piece and subjected in the electrolyte to anodic oxidation under the conditions and parameters set forth in the following table, the voltage between the anode and cathode being regulated in known manner to maintain a constant current density:

| No. | Material        | Current density (a./dm. <sup>2</sup> ) | Voltage range |       | Temperature of solution (°C.) | Time of anodizing (min.) |
|-----|-----------------|----------------------------------------|---------------|-------|-------------------------------|--------------------------|
|     |                 |                                        | Starting      | Final |                               |                          |
| 1   | 1080 (99.8% Al) | 2                                      | 65            | 84    | 16-18                         | 45                       |
| 2   | 5052 (52 S)     | 2                                      | 62            | 95    | 17.5-18                       | 45                       |
| 3   | 6063 (63 S)     | 2                                      | 63            | 88    | 18-20                         | 45                       |

Set forth in the following table are the properties of the anodic oxidation coatings formed on the respective samples, treated as above:

| No. | Material        | Film thickness (μ) | Abrasion resistance |        | Color                         |
|-----|-----------------|--------------------|---------------------|--------|-------------------------------|
|     |                 |                    | Hardness (Hv)       | (sec.) |                               |
| 1   | 1080 (99.8% Al) | 18.5               | 552                 | 2,933  | Slightly yellowish deep gray. |
| 2   | 5052 (52 S)     | 16                 | 533                 | 5,773  | Dark olive.                   |
| 3   | 6063 (63 S)     | 23.8               | 536                 | 5,760  | Dark brown.                   |

For comparison purposes an electrolyte similar to that described above but without addition of sulfuric acid and having the following composition was prepared:

|                    | Grams/liter |
|--------------------|-------------|
| Acetamide          | 80          |
| Oxalic acid        | 10          |
| Water <sup>1</sup> | Balance     |

<sup>1</sup> 1 liter in total amount.

Employing the above electrolyte without sulfuric acid, three aluminum plate work pieces were treated in the manner described above under the following conditions and parameters:

| No. | Material        | Current density (a./dm. <sup>2</sup> ) | Voltage range |       | Temperature of solution (°C.) | Time of anodizing (min.) |
|-----|-----------------|----------------------------------------|---------------|-------|-------------------------------|--------------------------|
|     |                 |                                        | Starting      | Final |                               |                          |
| 1   | 1080 (99.8% Al) | 2                                      | 76            | 105   | 16-18                         | 45                       |
| 2   | 5052 (52 S)     | 2                                      | 77            | 115   | 16-19                         | 45                       |
| 3   | 6063 (63 S)     | 2                                      | 98            | 155   | 21-21                         | 45                       |

The properties of the anodic oxidation coatings of the last treated samples are as follows:

50 ions in aqueous solution whereby the sulfuric acid concentration is as specified, preferably in the range of 0.1

| No. | Material        | Film thickness (μ) | Abrasion resistance |        | Color                |
|-----|-----------------|--------------------|---------------------|--------|----------------------|
|     |                 |                    | Hardness (Hv)       | (sec.) |                      |
| 1   | 1080 (99.8% Al) | 20                 | 531                 | 4,270  | Pale yellowish gray. |
| 2   | 5052 (52 S)     | 16                 | 530                 | 5,472  | Olive.               |
| 3   | 6063 (63 S)     | 20                 | 493                 | 4,740  | Light brown.         |

As can be seen from the above examples, by employing the improved electrolyte composition in the anodic oxidation of aluminum surfaces a wide range of colors is available in deep hues. As compared to an electrolyte which differs from the improved electrolyte only in the omission of the sulfate ion, its use provides much darker shades under identical current and time treating parameters and the voltage required for the same current densities are considerably less with the improved electrolyte resulting in a reduction in power consumption and equipment and installation costs. It should be noted, that as the coating on the work piece builds up, the resistance between the electrodes increases thereby necessitating an increase in the interelectrode voltage to maintain a constant current density. This control may be manually performed but is preferably accomplished automatically by known electrical regulator networks so that the current density does not vary during the full treatment period

5 whereby to optimumly obtain the desired color and coating.

10 The color of the anodized coating depends on the composition of the work piece. The thicker the oxidized coating, the deeper the color becomes, so that by supplying the current selectively for an appropriate period of time, desired coloration can be achieved through a single step of anodic oxidation. In addition, the coating obtained with the use of the improved electrolyte is tough and high in wear resistance and is substantially free of any pores. (Pinhole test results in no deposition of copper

20 other than by corner effect.) It also has excellent resistance to light and weather-proof property and does not develop cracks even when it is thick. The oxidized coat-

30 ing in accordance with the present invention can be formed in a wider range of colors which covers deeper colors as compared with the coating produced by anodic oxidation which utilizes an aqueous solution consisting of acetamide and oxalic acid. The higher the ratio of the amount of acetamide to that of oxalic acid, the darker color of the oxidized article is attained.

35 The improved electrolyte set forth above may be modified as earlier described by varying the concentrations of the acetamide, oxalic acid, and sulfuric acid or sulfate ion in the manner earlier described. The sulfuric acid may be substituted in whole or in part by a water soluble sulfate salt or compound which provides sulfate

60 ions in aqueous solution whereby the sulfuric acid concentration is as specified, preferably in the range of 0.1

to 2.0 grams per liter of electrolyte solution. An example of a suitable sulfate compound is nickle sulfate, or the like.

65 While there have been described preferred embodiments of the present invention, it is apparent that numerous alterations, omissions and additions may be made without departing from the spirit thereof.

What is claimed is:

1. An electrolyte for the anodic oxidation of aluminum and alloys thereof comprising an aqueous solution containing by weight of said electrolyte, 1% to 50% of acetamide, 0.1% to 10% of oxalic acid, and 0.01% to 0.5% of sulphuric acid or its molal equivalent of a water soluble sulphate or combination thereof with sulfuric acid.

70 2. The electrolyte of claim 1 wherein said electrolyte contains 30 to 200 grams per liter of said acetamide, 3 to 30 grams per liter of said oxalic acid, and 0.1 to 2 grams per liter of said sulfuric acid or the molal equiv-

alent thereof of a water soluble sulfate or a combination thereof with sulfuric acid.

3. The method of treating an aluminum containing work piece comprising immersing said work piece as the anode and immersing a cathode in the electrolyte of claim 1 and applying a voltage between said work piece and said cathode of a value sufficient to form an oxidation coating on said work piece.

4. The method of claim 3 wherein said voltage is increased during said treatment.

5. The method of claim 3 wherein the initial voltage applied between said work piece and electrode is below 70 volts.

6. The method of claim 3 wherein the temperature of said electrolyte is between 15° C. and 25° C.

#### References Cited

#### UNITED STATES PATENTS

3,472,744 10/1969 Kape ----- 204—58

#### OTHER REFERENCES

10 "The Anodizing of Aluminum in Electrolytes Based on Organic Solvents," Plating, January 1968, pp. 26—34.

JOHN H. MACK, Primary Examiner

R. L. ANDREWS, Assistant Examiner